



US010202820B2

(12) **United States Patent**  
**Xu et al.**

(10) **Patent No.:** **US 10,202,820 B2**  
(45) **Date of Patent:** **Feb. 12, 2019**

(54) **HIGH STRENGTH, FLOWABLE, SELECTIVELY DEGRADABLE COMPOSITE MATERIAL AND ARTICLES MADE THEREBY**

(71) Applicants: **Zhiyue Xu**, Cypress, TX (US); **Bobby J. Salinas**, Houston, TX (US); **Zhihui Zhang**, Katy, TX (US)

(72) Inventors: **Zhiyue Xu**, Cypress, TX (US); **Bobby J. Salinas**, Houston, TX (US); **Zhihui Zhang**, Katy, TX (US)

(73) Assignee: **BAKER HUGHES, A GE COMPANY, LLC**, Houston, TX (US)

(\*) Notice: Subject to any disclaimer, the term of this patent is extended or adjusted under 35 U.S.C. 154(b) by 535 days.

(21) Appl. No.: **14/573,721**

(22) Filed: **Dec. 17, 2014**

(65) **Prior Publication Data**

US 2016/0177661 A1 Jun. 23, 2016

(51) **Int. Cl.**

**C22C 29/00** (2006.01)  
**E21B 33/13** (2006.01)

(Continued)

(52) **U.S. Cl.**

CPC ..... **E21B 33/13** (2013.01); **C22C 1/0458** (2013.01); **C22C 1/058** (2013.01); **C22C 29/005** (2013.01);

(Continued)

(58) **Field of Classification Search**

CPC ... B22F 2998/10; C22C 1/0458; C22C 1/058; C22C 29/005; C22C 29/06;

(Continued)

(56) **References Cited**

U.S. PATENT DOCUMENTS

2005/0272846 A1 12/2005 Price et al.  
2011/0132143 A1 6/2011 Xu et al.

(Continued)

OTHER PUBLICATIONS

Petr Vanysek, *Electrochemical Series, CRC Handbook of Chemistry and Physics, Internet Version, 2017*, pp. 5-78 to 5-84.\*

(Continued)

*Primary Examiner* — Scott R Kastler

*Assistant Examiner* — Vanessa T. Luk

(74) *Attorney, Agent, or Firm* — Cantor Colburn LLP

(57) **ABSTRACT**

A lightweight, selectively degradable composite material includes a compacted powder mixture of a first powder and a second powder. The first powder comprises first metal particles comprising Mg, Al, Mn, or Zn, having a first particle oxidation potential. The second powder comprises low-density ceramic, glass, cermet, intermetallic, metal, polymer, or inorganic compound second particles. At least one of the first particles and the second particles includes a metal coating layer of a coating material disposed on an outer surface having a coating oxidation potential that is different than the first particle oxidation potential. The compacted powder mixture has a microstructure comprising: a matrix comprising the first metal particles; the second particles dispersed within the matrix; and a network comprising interconnected adjoining metal coating layers that extends throughout the matrix, the lightweight, selectively degradable composite material having a density of about 3.5 g/cm<sup>3</sup> or less.

**36 Claims, 5 Drawing Sheets**



| (51) <b>Int. Cl.</b>                                                                                                                                                                                                                                                                                                                                                                                     | (56) <b>References Cited</b>                                                                                                                                                                                     |
|----------------------------------------------------------------------------------------------------------------------------------------------------------------------------------------------------------------------------------------------------------------------------------------------------------------------------------------------------------------------------------------------------------|------------------------------------------------------------------------------------------------------------------------------------------------------------------------------------------------------------------|
| <i>C22C 29/02</i> (2006.01)                                                                                                                                                                                                                                                                                                                                                                              |                                                                                                                                                                                                                  |
| <i>C22C 29/12</i> (2006.01)                                                                                                                                                                                                                                                                                                                                                                              |                                                                                                                                                                                                                  |
| <i>C22C 29/16</i> (2006.01)                                                                                                                                                                                                                                                                                                                                                                              |                                                                                                                                                                                                                  |
| <i>C22C 29/18</i> (2006.01)                                                                                                                                                                                                                                                                                                                                                                              |                                                                                                                                                                                                                  |
| <i>C22C 32/00</i> (2006.01)                                                                                                                                                                                                                                                                                                                                                                              |                                                                                                                                                                                                                  |
| <i>C22C 49/06</i> (2006.01)                                                                                                                                                                                                                                                                                                                                                                              | 2012/0080189 A1 4/2012 Marya et al.                                                                                                                                                                              |
| <i>C22C 49/11</i> (2006.01)                                                                                                                                                                                                                                                                                                                                                                              | 2013/0028781 A1* 1/2013 Xu ..... B22F 1/02<br>419/48                                                                                                                                                             |
| <i>C22C 49/14</i> (2006.01)                                                                                                                                                                                                                                                                                                                                                                              |                                                                                                                                                                                                                  |
| <i>E21B 33/12</i> (2006.01)                                                                                                                                                                                                                                                                                                                                                                              | 2013/0052472 A1 2/2013 Xu                                                                                                                                                                                        |
| <i>C22C 1/04</i> (2006.01)                                                                                                                                                                                                                                                                                                                                                                               | 2013/0248183 A1* 9/2013 Pisklak ..... C09K 8/428<br>166/292                                                                                                                                                      |
| <i>C22C 1/05</i> (2006.01)                                                                                                                                                                                                                                                                                                                                                                               |                                                                                                                                                                                                                  |
| <i>C22C 29/06</i> (2006.01)                                                                                                                                                                                                                                                                                                                                                                              | 2013/0299185 A1* 11/2013 Xu ..... E21B 43/106<br>166/376                                                                                                                                                         |
|                                                                                                                                                                                                                                                                                                                                                                                                          | 2014/0228972 A1 8/2014 Xu                                                                                                                                                                                        |
| (52) <b>U.S. Cl.</b>                                                                                                                                                                                                                                                                                                                                                                                     |                                                                                                                                                                                                                  |
| CPC ..... <i>C22C 29/02</i> (2013.01); <i>C22C 29/06</i> (2013.01); <i>C22C 29/05</i> (2013.01); <i>C22C 29/12</i> (2013.01); <i>C22C 29/16</i> (2013.01); <i>C22C 29/18</i> (2013.01); <i>C22C 32/001</i> (2013.01); <i>C22C 32/0047</i> (2013.01); <i>C22C 49/06</i> (2013.01); <i>C22C 49/11</i> (2013.01); <i>C22C 49/14</i> (2013.01); <i>E21B 33/1208</i> (2013.01); <i>B22F 2998/10</i> (2013.01) |                                                                                                                                                                                                                  |
| (58) <b>Field of Classification Search</b>                                                                                                                                                                                                                                                                                                                                                               |                                                                                                                                                                                                                  |
| CPC ..... C22C 29/065; C22C 29/02; C22C 29/12; C22C 29/16; C22C 29/18; C22C 32/001; C22C 32/0047; C22C 49/06; C22C 49/11; C22C 49/14; E21B 33/13; E21B 33/1208                                                                                                                                                                                                                                           |                                                                                                                                                                                                                  |
| See application file for complete search history.                                                                                                                                                                                                                                                                                                                                                        |                                                                                                                                                                                                                  |
|                                                                                                                                                                                                                                                                                                                                                                                                          | <b>U.S. PATENT DOCUMENTS</b>                                                                                                                                                                                     |
|                                                                                                                                                                                                                                                                                                                                                                                                          | “Properties of Pure Metals,” Properties and Selection: Nonferrous Alloys and Special-Purpose Materials, vol. 2, ASM Handbook, ASM International, 1990, pp. 1099-1201 (print version), 6 pages (online version).* |
|                                                                                                                                                                                                                                                                                                                                                                                                          | Aluminum-Matrix Composites, Metal-Matrix Composites, Metals Handbook Desk Edition, ASM International, 1998, pp. 674-680 (print version), 14 pages total (online version). (Year: 1998).*                         |
|                                                                                                                                                                                                                                                                                                                                                                                                          | International Search Report for International Application No. PCT/US2015/061202 dated Feb. 17, 2016.                                                                                                             |
|                                                                                                                                                                                                                                                                                                                                                                                                          | Written Opinion for International Application No. PCT/US2015/061202 dated Feb. 17, 2016.                                                                                                                         |
|                                                                                                                                                                                                                                                                                                                                                                                                          | Han, et al., “Mechanical Properties of Nanostructured Materials”, Rev. Adv. Mater. Sci. 9(2005) 1-16.                                                                                                            |
|                                                                                                                                                                                                                                                                                                                                                                                                          | * cited by examiner                                                                                                                                                                                              |



FIG. 1A





FIG. 2A



FIG. 2B



FIG. 3A



FIG. 3B



FIG. 4A



FIG. 4B



FIG. 5C



FIG. 6

## 1

**HIGH STRENGTH, FLOWABLE,  
SELECTIVELY DEGRADABLE COMPOSITE  
MATERIAL AND ARTICLES MADE  
THEREBY**

BACKGROUND

Oil and natural gas wells often utilize wellbore components or tools that, due to their function, are only required to have limited service lives that are considerably less than the service life of the well. After a component or tool service function is complete, it must be removed or disposed of in order to recover the original size of the fluid pathway for use, including hydrocarbon production, CO<sub>2</sub> sequestration, etc. Disposal of components or tools has conventionally been done by milling or drilling the component or tool out of the wellbore, which are generally time consuming and expensive operations.

Recently, in order to improve well operations and reduce costs by reducing the need for milling or drilling operations, various interventionless, selectively removable wellbore components or tools have been developed. These selectively removable components or tools include or are formed from various dissolvable, degradable, corrodible, or otherwise removable materials and can be removed from a wellbore without mechanical intervention, such as by changing the conditions in the wellbore, including the temperature, pressure or chemical constituent makeup of a wellbore fluid. While these materials are very useful, it is also very desirable that these materials be lightweight and have high strength, including a strength comparable to that of conventional engineering materials used to form wellbore components or tools, such as various grades of steel, stainless steel and other Ni-base, Co-base and Fe-base alloys. As an example, Fe-base selectively removable materials have been developed. These Fe-base removable materials are high strength and have an ultimate compressive strength of about 100 ksi at room temperature and a density of about 5.3 g/cm<sup>3</sup>. While very useful, these materials are not ideal for use in certain applications, such as in horizontal portions of the wellbore, because they are more dense than the wellbore fluids and have a tendency to settle out of the fluid requiring higher fluid pressures to affect their movement or run-in into horizontal portions of the wellbore.

While it is very desirable to use selectively removable components and tools in all portions of a well, selectively removable components and tools are particularly desirable for use in horizontal portions of the well, since a single vertical well may include a plurality of horizontal portions at a given depth, and this plurality of horizontal portions may be established at a plurality of depths. The extensive and expanding use of horizontal drilling makes the development of improved high strength, lightweight, selectively removable materials very desirable.

Thus, the further improvement of high strength, lightweight, selectively removable materials and articles, including downhole tools and components, is very desirable.

SUMMARY

A lightweight, selectively degradable composite material includes a compacted powder mixture of a first powder and a second powder. The first powder comprises first metal particles comprising Mg, Al, Mn, or Zn, or an alloy of any of the above, or a combination of any of the above, having a first particle oxidation potential. The second powder comprises low-density ceramic, glass, cermet, intermetallic,

## 2

metal, polymer, or inorganic compound second particles. At least one of the first particles and the second particles includes a metal coating layer of a coating material disposed on an outer surface having a coating oxidation potential that is different than the first particle oxidation potential. The compacted powder mixture has a microstructure comprising: a matrix comprising the first metal particles; the second particles dispersed within the matrix; and a network comprising interconnected adjoining metal coating layers that extends throughout the matrix, the lightweight, selectively degradable composite material having a density of about 3.5 g/cm<sup>3</sup> or less.

BRIEF DESCRIPTION OF THE DRAWINGS

15 Referring now to the drawings wherein like elements are numbered alike in the several Figures:

FIG. 1A is a schematic cross-section of an embodiment of a well including vertical and horizontal portions configured for use of selectively degradable articles of the lightweight, high strength, degradable composite material disclosed herein;

FIG. 1B is an enlarged portion B of the well of FIG. 1A illustrating an embodiment of a degradable ball and an embodiment of a degradable seat, such as a ball seat, formed of the lightweight, high strength, degradable composite material disclosed herein;

FIG. 1C is a schematic cross-section of an embodiment of a degradable plug formed of the lightweight, high strength, degradable composite material disclosed herein;

FIG. 1D is a schematic cross-section of an embodiment of a degradable disk formed of the lightweight, high strength, degradable composite material disclosed herein;

FIG. 1E is a schematic cross-section of an embodiment of a degradable dart formed of the lightweight, high strength, degradable composite material disclosed herein;

FIG. 2A is a schematic illustration of an exemplary embodiment of a powder mixture 10 comprising first powder 20 and second powder 30;

FIG. 2B is a schematic illustration of an exemplary embodiment of a powder compact 100 of powder mixture 10 of FIG. 2A;

FIG. 3A is a schematic illustration of a second exemplary embodiment of a powder mixture 10 comprising first powder 20 and second powder 30;

FIG. 3B is a schematic illustration of an exemplary embodiment of a powder compact 100 of powder mixture 10 of FIG. 3A;

FIG. 4A is a schematic illustration of a third exemplary embodiment of a powder mixture 10 comprising first powder 20 and second powder 30;

FIG. 4B is a schematic illustration of an exemplary embodiment of a powder compact 100 of powder mixture 10 of FIG. 4A;

FIG. 5A is an electron photomicrograph of an exemplary embodiment of a powder mixture 10;

FIG. 5B is a backscatter electron photomicrograph of an exemplary embodiment of a powder compact 110 of the powder mixture 10;

FIG. 5C is a plot of stress as a function of strain in an embodiment of the powder compact 110; and

FIG. 6 is a secondary electron photomicrograph of another exemplary embodiment of the powder compact 110.

DETAILED DESCRIPTION

65 Referring to the figures, and particularly FIGS. 1B-6, a lightweight, high strength, flowable, selectively degradable

composite material 100 is disclosed. The selectively degradable composite material 100 has a high strength, such as an Ultimate Compressive Strength (UCS) of at least about 80 ksi, and in certain embodiments an even higher strength, including an ultimate compressive strength of at least about 100 ksi. Advantageously, the selectively degradable composite materials 100 described herein have a high strength comparable to that of Fe-base removable materials, as described herein, and a lower density. As a further advantage, the selectively degradable composite materials 100 are lightweight, including having a selectively controllable density of about 1.5 to about 3.5 g/cm<sup>3</sup>, and more particularly about 2.0 to about 3.5 g/cm<sup>3</sup>, and even more particularly about 2.0 to about 3.0 g/cm<sup>3</sup>. The selectively controllable density described herein enables selection of a density of the composite material 100, as well as articles that include or are formed from the composite material, which allows the material or article to be flowable with the wellbore, particularly within horizontal portions of the wellbore 2 (FIGS. 1A and 1B). FIGS. 1A and 1B illustrate a well 1 and wellbore 2 that includes horizontal portions 4 and vertical portions 5. One problem associated with operations in the horizontal portions 4 of the wellbore 2 is that tools 230 and components 240 that are to be run in with a particular wellbore fluid 6 often have a density that is greater than the density of the wellbore fluid 6, such that they have a tendency to settle out of the flow 11 of the wellbore fluid 6 against the downward-most portion 7 of the wellbore (e.g. the lowest portion of the inner diameter of the well casing 8 in a cased well 1), which tendency requires accommodation in the material/article design as well as the design of the processes and operations for which they are used, such as the use of higher wellbore fluid 6 working pressures P and flow 11 rates, for example. The composite materials disclosed herein are very advantageous and enable a method of using degradable downhole articles 220 that is particularly advantageous because it enables run in of these articles under conditions where the tendency of the article to settle, particularly in horizontal portion 4 is greatly reduced or eliminated by using downhole articles, including downhole tools 230 and components 240, having a density that is close to or even substantially equal to, including equal to, the density of the wellbore fluid 6 used to run it in, such that the buoyancy characteristics and buoyant forces on the articles described herein may be achieved. The wellbore fluids 6 may be any suitable wellbore fluids 6, including naturally occurring formation fluids 9, such as those that are extracted from or may be accessed from the earth formation 3 in which the well 1 is placed, and wellbore fluids 6 of any type that are introduced into the wellbore 2 from the surface, such as various drilling, completion and production wellbore fluids 6, or combinations of formation fluids 9 and surface wellbore fluids 13. This may include any number of ionic fluids and/or highly polar fluids, such as those that contain various chlorides, including all manner of fresh or salt water, brines and oil bearing fluids. Examples include potassium chloride (KCl), hydrochloric acid (HCl), calcium chloride (CaCl<sub>2</sub>), calcium bromide (CaBr<sub>2</sub>), or zinc bromide (ZnBr<sub>2</sub>), or combinations thereof. The wellbore fluids 6 may be composite fluids that include solids dispersed or suspended or gelled in any manner within the fluid, such as formation materials, sand, proppants and the like, for example. These fluids, or composite fluids, may have a density of about 1.0 to about 3.5 g/cm<sup>3</sup>, and more particularly about 1.5 to about 3.5 g/cm<sup>3</sup>, and even more particularly about 2.0 to about 3.5 g/cm<sup>3</sup>, and even more particularly about 2.0 to about 3.0 g/cm<sup>3</sup>. The selectively controllable density of the selectively degradable

composite material 100 allows the material, and articles 200 made from the material, to have a density that is selected in conjunction with the selection of the wellbore fluid 6 being used, or vice versa, to provide a selectable buoyancy of the material and/or article that reduces, or in some embodiments eliminates, its tendency to settle in the wellbore fluid 6. For example, in certain embodiments the selectively controllable density of the composite material 100 and/or article 200 may be selected to provide positive, neutral, or negative buoyancy, and more particularly may be selected to provide a buoyancy that is just slightly negative or slightly positive, such that the material and/or article has a tendency to slowly sink or slowly rise in the fluid, respectively, in a particular or predetermined wellbore fluid 6. For example, the density of the selectively degradable composite material and the wellbore fluid 6 may be selected to be the same to provide neutral buoyancy. In another example, the density of the selectively degradable composite material and the wellbore fluid 6 may be selected to be slightly positive or negative buoyancy by establishing a predetermined positive or negative buoyancy force differential of the material and/or article in the wellbore fluid 6, where the wellbore fluid may have any suitable density, including a density of about 1 to about 2.5 g/cc. Thus, the present invention is very advantageous by reducing the fluid pressures P or flow 11 rate needed to run in the composite material 100 and/or downhole articles 220 made from the composite material into the wellbore 2, particularly horizontal portions 4 of the wellbore, while offering the flexibility of selective degradation and removal from the wellbore once its intended function has been performed. As an example, a ball 300, or similarly a plug 310 (FIG. 1C), disk 320 (FIG. 1D), dart 330 (FIG. 1E) or other downhole article 220 of the degradable composite material 100 can be run in to the wellbore 2, particularly horizontal portions 4 of the wellbore, in a selected or predetermined wellbore fluid 6 where the article and fluid are selected to provide predetermined buoyancy force differential and reduce the run in fluid pressure P and/or flow 11 requirements, such as, for example, reducing a fluid pressure differential required to move a moveable article (e.g. a ball, plug or dart in the wellbore fluid and/or reduce an impact force when landing in or on a horizontal leg. The article can be sealably seated against a degradable seat 340 formed from the degradable composite material 100 to perform a wellbore operation, such as a fracking operation as shown in FIG. 1A, and can then be selectively degraded, including selective removal, by a subsequent wellbore operation such as an acidizing operation, for example. The lightweight, selectively degradable composite material 100 includes a powder compact 110 of powder mixture 10 of a first powder 20 and a second powder 30. The first powder 20 comprises first metal particles 22 comprising Mg, Al, Mn, or Zn, or an alloy of any of the above, or a combination of any of the above, having a first particle oxidation potential. The second powder 30 comprises low-density, lightweight, high strength ceramic, glass, cermet, intermetallic, metal, polymer, or inorganic compound second particles 32. At least one of the first metal particles 22 and the second particles 32 includes a metal coating layer 40 of a coating material 42 disposed on an outer surface having a coating oxidation potential that is different than the first particle oxidation potential. The compacted powder mixture 10 has a microstructure 50 comprising: a matrix 52 comprising the deformed and compacted first metal particles 22; the second particles 32 dispersed within the matrix 52 as dispersed particles 54; and a network 56 comprising interconnected adjoining metal coating layers 40 that are joined

or bonded by the compaction and associated deformation and extends throughout the matrix **52**. The lightweight, selectively degradable composite material **100** has a density of about 3.5 g/cm<sup>3</sup> or less, as described herein. This micro-structure **50** is very advantageous because the network **56** of the coating material **34** that extends throughout and is metallurgically bonded within and to the matrix **52** of the first metal particles **22** provides an oxidation potential difference between these materials that extends throughout the composite material. The oxidation potential difference between the coating material **42** and the matrix **52** of the compacted and metallurgically bonded first metal particles **22** provides for rapid degradation and removal of the composite material **100**, such as, for example, rapid dissolution or corrosion of the more anodic material in a predetermined wellbore fluid **6**. The rapid degradation and removal of the composite material **100** may also be enhanced by other predetermined wellbore conditions, including selection of a predetermined wellbore temperature and/or a predetermined wellbore pressure that triggers or enhances or accelerates the degradation. This invention discloses a new lightweight, selectively degradable composite material **100** and method of making and use. This lightweight, selectively degradable composite material encompasses high strength (e.g. a UCS of at least about 80 ksi, and in some embodiments at least about 100 ksi) and a controlled degradation, or dissolution, and/or disintegration rate while maintaining a low density (e.g. about 1.5 to about 3.5 g/cm<sup>3</sup>). Low density is achieved by introducing high strength, light weight, nano- or micro-size, solid or hollow particles in the system. The ultrahigh strength characteristic provides the high pressure rating of the downhole tools **230** or components **240** and the lightweight characteristic guarantees the buoyancy of the tools in a wellbore fluid **6**, both of which are imperative for down-hole applications, particularly horizontal downhole applications, such as flow control devices including frac balls **300**, darts **340**, disks **330** or plugs **320** and associated sealing seats **340**, for example.

The microstructure of the selectively degradable composite material is different from selectively degradable nano-matrix materials, such as those taught in US Patent Publication US2011/0132143A1, US2011/0135953A1, US2011/0135530A1, US2011/0136707A1, US2013/0047785A1, US2013/0052472A1, and US2013/0047784A1, which are incorporated herein by reference in their entirety, because it either does not have a substantially continuous cellular nanomatrix with dispersed metal particles, or because it includes dispersed lightweight (i.e. low density) particles. Rather, in the embodiments of the present invention, the interaction and joining or interconnection of the metal coating layers **40** of adjoining particles form a network **56**, which may be partially continuous, locally continuous or discontinuous, or a combination thereof, as described herein.

The powder mixtures **10** of first powder **20** and second powder **30** described herein may be formed in any suitable manner, including all manner of mechanical mixing, including various powder mills and blenders. In one embodiment, the powder mixture **10** is substantially homogeneous mixture, and more particularly a homogeneous mixture, where the first powder **20** particles and second powder **30** particles are substantially uniformly dispersed or uniformly dispersed, respectively, within one another. As used herein, substantially homogeneous means that there is uniformity within substantial portions of the mixture, but that there may be localized instances of non-uniformity within the mixture. In other embodiments, the powder mixture **10** may be heterogeneous mixtures of first powder **20** and second

powder **30**, including gradient mixtures of these particles analogous to the particle mixtures used to form functionally gradient articles as described in US Patent Publication US20120276356A1, which is incorporated herein by reference in its entirety.

In one embodiment, as illustrated in FIGS. 2A and 2B, the lightweight, high strength, selectively degradable composite material **100** is a powder compact material **110** formed by compacting powder mixture **10** of first powder **20** and second powder **30**. The first powder **20** comprises first metal particles **22**. The first metal particles **22** comprise Mg, Al, Mn, or Zn, or an alloy of any of the above, or a combination of any of the above. The first powder **20** and first metal particles **22** have a first particle oxidation potential. The second powder **30** comprises second particles **32**. The second particles **32** comprises low-density ceramic, glass, cermet, intermetallic, metal, polymer, or inorganic compound second particles **32**. At least one of the first metal particles **22** and the second particles **32** comprises a metal coating layer **40** of a coating material **42** disposed on an outer surface having a coating oxidation potential that is different than the first particle oxidation potential. In the embodiment of FIGS. 2A and 2B, the metal coating layer **40** is disposed on the outer surfaces **26** of the first metal particles **22**. In this embodiment, the metal coating layer **40** may be disposed on all of the first metal particles **22**, or alternately, the metal coating layer **40** may be disposed on only a portion of the first metal particles **22**, where the coated and uncoated first metal particles may be used in any suitable proportion. In this embodiment, the powder compact material **110** comprises compacted powder mixture **10** having a microstructure **50** comprising: a matrix **52** comprising the compacted first metal particles **22**. The microstructure also comprises the second particles **32** as dispersed particles **54** within the matrix **52**. The microstructure also comprises a network **56** comprising interconnected adjoining metal coating layers **40**, particularly metal coating layers **40** of adjoining first metal particles that are proximate one another and joined to one another in conjunction with compaction to form the powder compact **110**, which extends throughout the matrix **52**. In certain embodiments, particularly where the powder mixture **10** comprises relatively larger amounts, larger sizes, or both of first metal particles **22** the network **56** may be a partially continuous network where the metal coating layers **40** of a number of adjacent first metal particles **22** are joined to one another beyond immediately adjacent particles, such that the continuity extends beyond immediately adjacent first metal particles to establish a partially continuous network of metal coating layers **40** that may extend 50 or more particle diameters, and more particularly 100 or more particle diameters, and even more particularly 1000 or more particle diameters of first metal particles **22**. This may be measured, for example, by measuring the length of continuous metal layers **40** in a metallographic section to ensure that it extends more than two particle diameters, for example. Depending on the extent of the continuity, the partially continuous network **56** may also be described as locally continuous. For example, if the partial continuity of the network **56** extends only to metal coating layers **40** of immediately adjacent first metal particles **22**, or to a small cluster of immediately adjacent first metal particles **22**, the network **56** of metal coating layers may be said to be locally continuous, such as for example, if the network **56** of metal coating layers extends about 2 to less than about 50 particle diameters, and more particularly about 2 to about 30 particle diameters, and even more particularly about 2 to about 10 particle diameters of first metal particles. Local continuity of

network **56** may be affected, for example, where the first metal particles **22** includes a mixture of coated first metal particles **22** that include metal coating layer **40** and uncoated first metal particles **22**. In other embodiments, the network **56** may be substantially discontinuous, including discontinuous, where continuity of the metal coating layers **40** does not extend substantially beyond or beyond, respectively, immediately adjacent first powder particles **22**, such that the first metal particles **22** with coating layers **40** are isolated and not joined to one another. A discontinuous network **56** may be affected, for example, where the first metal particles **22** include a mixture of coated first metal particles **22** that include metal coating layer **40** and uncoated first metal particles **22**, particularly where the proportion of uncoated particles is greater than that of the coated particles. In this embodiment, the first metal particles **22** and second particles **32** may be present in any suitable amounts. In one embodiment, the first metal particles include about 10 to about 50 percent, and the second particles **32** include about 50 to about 90 percent, and the coating layers comprise about 0.5 to about 5 percent, by weight of the composite material **100**, and in another embodiment the first metal particles include about 15 to about 50 percent, and the second particles **32** include about 50 to about 85 percent, and the coating layers comprise about 0.5 to about 5 percent, by weight of the composite material **100**. The lightweight, selectively degradable composite material **100** has a density of about 3.5 g/cm<sup>3</sup> or less, as described herein.

In another embodiment, as illustrated in FIGS. 3A and 3B, the lightweight, high strength, selectively degradable composite material **100** is a powder compact material **110** formed by compacting powder mixture **10** of first powder **20** and second powder **30**. The first powder **20** comprises first metal particles **22**. The first metal particles **22** comprise Mg, Al, Mn, or Zn, or an alloy of any of the above, or a combination of any of the above. The first powder **20** and first metal particles **22** have a first particle oxidation potential. The second powder **30** comprises second particles **32**. The second particles **32** comprise low-density ceramic, glass, cermet, intermetallic, metal, polymer, or inorganic compound second particles **32**. At least one of the first metal particles **22** and the second particles **32** comprises a metal coating layer **40** of a coating material **42** disposed on an outer surface having a coating oxidation potential that is different than the first particle oxidation potential. In the embodiment of FIGS. 3A and 3B, the metal coating layer **40** is disposed on the outer surfaces **36** of the second particles **32**. In this embodiment, the metal coating layer **40** may be disposed on all of the second particles **32**, or alternately, the metal coating layer **40** may be disposed on only a portion of the second particles **32**, where the coated and uncoated second particles may be used in any suitable proportion. In this embodiment, the powder compact material **110** comprises compacted powder mixture **10** having a microstructure **50** comprising: a matrix **52** comprising the compacted first metal particles **22**. The microstructure also comprises the metal coated second particles **32** as dispersed particles **54** within the matrix **52**. In certain embodiments, where the amount of the metal coated second particles **32** is large enough, the microstructure also comprises a network **56** comprising interconnected adjoining metal coating layers **40**, particularly metal coating layers **40** of adjoining metal coated second particles **32** that are proximate one another and whose metal coating layers **40** are joined to one another in conjunction with compaction to form the powder compact **110**, which extends throughout the matrix **52**. In certain embodiments, particularly where the powder mixture **10**

comprises relatively larger amounts, larger sizes, or both of second particles **32** the network **56** may be a partially continuous network where the metal coating layers **40** of a number of adjacent second particles **32** are joined to one another beyond immediately adjacent particles, such that the continuity extends beyond immediately adjacent second particles **32** to establish a partially continuous network of metal coating layers **40** of these particles that may extend 50 or more particle diameters, and more particularly 100 or 10 more particle diameters, and even more particularly 1000 or more particle diameters of second particles **32**. This may be measured, for example, by measuring the length of continuous metal layers **40** in a metallographic section to ensure that it extends more than two particle diameters, for example. 15 Depending on the extent of the continuity, the partially continuous network **56** may also be described as locally continuous. For example, if the partial continuity of the network **56** extends only to metal coating layers **40** of immediately adjacent particles second particles **32**, or to a 20 small cluster of immediately adjacent second particles **32**, the network **56** of metal coating layers may be said to be locally continuous, such as for example, if the network **56** of metal coating layers **40** extends about 2 to less than about 50 particle diameters, and more particularly about 2 to about 30 particle diameters, and even more particularly about 2 to about 10 particle diameters of second particles **32**. Local continuity of network **56** may be affected, for example, where the second particles **32** includes a mixture of coated second particles **32** that include metal coating layer **40** and uncoated second particles **32**. In other embodiments, the network **56** may be substantially discontinuous, including discontinuous, where continuity of the metal coating layers **40** does not extend substantially beyond or beyond, respectively, immediately adjacent second particles **32**, such that the second particles **32** with coating layers **40** are isolated and not joined to one another. A discontinuous network **56** may be affected, for example, where the second particles **32** include a mixture of coated second particles **32** that include metal coating layer **40** and uncoated second particles **32**, particularly where the proportion of uncoated particles is greater than that of the coated particles. In this embodiment, the first metal particles **22** and second particles **32** may be present in any suitable amounts. In one embodiment, the first metal particles include about 10 to about 50 percent, and the second particles **32** include about 50 to about 90 percent, and the coating layers comprise about 0.5 to about 5 percent, by weight of the composite material **100**, and in another embodiment the first metal particles include about 15 to about 50 percent, the second particles comprise about 50 to about 85, and the coating layers comprise about 0.5 to about 5 percent, by weight of the composite material. The lightweight, selectively degradable composite material **100** has a density of about 3.5 g/cm<sup>3</sup> or less, as described herein.

In yet another embodiment, as illustrated in FIGS. 4A and 55 4B, the lightweight, high strength, selectively degradable composite material **100** is a powder compact material **110** formed by compacting powder mixture **10** of first powder **20** and second powder **30**. The first powder **20** comprises first metal particles **22**. The first metal particles **22** comprise Mg, 60 Al, Mn, or Zn, or an alloy of any of the above, or a combination of any of the above. The first powder **20** and first metal particles **22** have a first particle oxidation potential. The second powder **30** comprises second particles **32**. The second particles **32** comprise low-density ceramic, glass, cermet, intermetallic, metal, polymer, or inorganic compound second particles **32**. At least one of the first metal particles **22** and the second particles **32** comprises a metal

coating layer 40 of a coating material 42 disposed on an outer surface having a coating oxidation potential that is different than the first particle oxidation potential. In the embodiment of FIGS. 4A and 4B, the metal coating layer 40 is disposed on the outer surfaces 26 of the first metal particles 22 and the outer surfaces 36 of the second particles 32. In this embodiment, the metal coating layer 40 may be disposed on all of the first metal particles 22 and/or all of second particles 32, or alternately, the metal coating layer 40 may be disposed on only a portion of the first metal particles 22 and/or only a portion of the second particles 32, where the coated and uncoated first metal particles 22 and/or the coated and uncoated second particles 32 may be used in any suitable proportion. In one embodiment, the metal coating layers 40 disposed on the first metal particles 22 and the second particles 32 may be the same metal coating layers 40, including the same material, number of layers and thickness, and in another embodiment the metal coating layers 40 disposed on the first metal particles 22 and the second particles 32 may be different, including different materials, numbers of layers or thicknesses. In this embodiment, the powder compact material 110 comprises compacted powder mixture 10 having a microstructure 50 comprising: a matrix 52 comprising the compacted metal coated first metal particles 22. The microstructure also comprises the metal coated second particles 32 as dispersed particles 54 within the matrix 52. The microstructure 50 also comprises a network 56 comprising interconnected adjoining metal coating layers 40, particularly metal coating layers 40 of adjoining first metal particles and second particles that are proximate one another and joined to one another in conjunction with compaction to form the powder compact 110, which extends throughout the matrix 52. In certain embodiments, particularly where the powder mixture 10 comprises relatively larger amounts, larger sizes, or both of first metal particles 22 the network 56 may be a partially continuous network where the metal coating layers 40 of a number of adjacent first metal particles 22 are joined to one another beyond immediately adjacent particles and/or to the metal coating layers of second particles, such that the continuity of the metal coating layers 40 extends beyond immediately adjacent first metal particles 22 and/or second particles 32 to establish a partially continuous network of metal coating layers 40 that may extend 50 or more particle diameters, and more particularly 100 or more particle diameters, and even more particularly 1000 or more particle diameters of first metal particles 22 or second particles 32. This may be measured, for example, by measuring the length of continuous metal layers 40 in a metallographic section to ensure that it extends more than two particle diameters, for example. Depending on the extent of the continuity, the partially continuous network 56 may also be described as locally continuous. For example, if the partial continuity of the network 56 extends only to metal coating layers 40 of immediately adjacent first metal particles 22 or second particles 32, or to a small cluster of immediately adjacent first metal particles 22 or second particles 32, the network 56 of metal coating layers may be said to be locally continuous, such as for example, if the network 56 of metal coating layers 40 extends about 2 to less than about 50 particle diameters, and more particularly about 2 to about 30 particle diameters, and even more particularly about 2 to about 10 particle diameters of first metal particles 22 or second particles 32. Local continuity of network 56 may be affected, for example, where the second particles 32 includes a mixture of coated second particles 32 that include metal coating layer 40 and uncoated second particles 32. In other

embodiments, the network 56 may be substantially discontinuous, including discontinuous, where continuity of the metal coating layers 40 does not extend substantially beyond or beyond, respectively, immediately adjacent first metal particles 22 and second particles 32, such that the first metal particles and second particles 32 with coating layers 40 are isolated and not joined to one another. A discontinuous network 56 may be affected, for example, where the first metal particles 22 and/or second particles 32 include a mixture of coated first metal particles and/or second particles 32 that include metal coating layer 40 and uncoated first metal particles 22 and/or second particles 32, particularly where the proportion of uncoated particles of either or both particle types is greater than that of the coated particles. In this embodiment, the first metal particles 22 and second particles 32 may be present in any suitable amounts. In one embodiment, the first metal particles include about 10 to about 50 percent, and the second particles 32 include about 50 to about 90 percent, and the coating layers comprise about 0.5 to about 5 percent, by weight of the composite material 100, and in another embodiment the first metal particles 22 comprise about 15 to about 50 percent, the second particles comprise about 50 to about 85 percent, and the coating layers comprise about 0.5 to about 5 percent, by weight of the composite material 100. It should be noted that even though the relative amounts of the first metal particles 22, second particles 32 and metal coating layers 40 may be the same as in the other embodiments (e.g. those of FIGS. 2A/2B and FIGS. 3A/3B) described herein, the strength, rate of degradation or corrosion in a wellbore fluid or other properties may be different from the materials of these embodiments due to differences in the distribution of the constituents with the resultant microstructures. The lightweight, selectively degradable composite material 100 has a density of about 3.5 g/cm<sup>3</sup> or less, as described herein.

The first metal particles 22 include Mg, Al, Mn, or Zn, or an alloy of any of the above, or a combination of any of the above. The first metal particles 22 may have any suitable size or shape. In one embodiment, the first metal particles 22 have an average size of about 5 to about 300 µm, and more particularly an average size of about 75 to about 150 µm. In one embodiment, the first metal particles 22 comprise a magnesium-base alloy. The magnesium-base alloy may include any suitable magnesium-base alloy, including an Mg—Si, Mg—Al, Mg—Zn, Mg—Mn, Mg—Al—Zn, Mg—Al—Mn, Mg—Zn—Zr, or Mg—X alloy, where X comprises a rare earth element, or an alloy of thereof, or any other combination of the aforementioned alloys. As used herein, rare earth elements include Sc, Y, La, Ce, Pr, Nd, or Er, or a combination of rare earth elements.

The second particles 32 may include any suitable low density particle. In one embodiment the second particles 32 include low-density ceramic, glass, cermet, intermetallic, metal, polymer, or inorganic compound second particles 32.

The second particles 32 may have any suitable size or shape. In one embodiment, the second particles 32 have a density of about 0.1 to about 4.5 g/cm<sup>3</sup>. The metal particles may include any suitable metal particles, including hollow or porous metal particles. In one embodiment, the metal particles may include pure titanium particles. In another embodiment the metal particles may include titanium alloy particles. Titanium alloy particles may include particles of any suitable commercially available titanium alloy or grade (e.g. Grades 1-38), including, for example, Ti-6Al-4V, which has a nominal composition comprising, by weight: about 6 percent aluminum, about 4 percent vanadium, and the balance

titanium and incidental impurities. In another embodiment, the metal particles include hollow metal particles, particularly hollow iron alloy particles, and more particularly hollow iron-base alloy particles, and even more particularly hollow steel particles. In one embodiment, the metal particles may have an average particle size of about 10 to about 200  $\mu\text{m}$ . The use of metal particles as second particles 32 is highly advantageous because while providing low density, lightweight powder compacts 100 as described herein, the powder compact materials 110 made using metal particles as second particles 32 are also capable of being rapidly formed to a near-net shape, such as by dynamic forging, which is highly desirable. In addition, powder compact materials 110 made using metal particles as second particles 32 are metallic materials and are also readily formable and/or machinable using any of a number of commercial metal working and finishing processes to a final or net shape. They may, for example, be finished to precise tolerances and surface finishes, which is useful in the manufacture of articles from these materials that require mating seating and/or sealing surfaces, such as balls, plugs, darts and the like that have mating seating and/or sealing surfaces. In addition to being lightweight and high strength, as described herein, the powder compact materials 110 made using metal particles as second particles 32 are also capable of providing relatively higher ductility and fracture toughness. In another embodiment, the second particles 32 include ceramic, glass, polymer, or inorganic compound particles, including hollow or porous particles of these materials. In another embodiment, the second particles 32 include ceramic particles comprising metal carbide, nitride, or oxide particles, or a combination thereof. One embodiment of ceramic particles includes silicon carbide particles, and more particularly silicon carbide particles that have an average particle diameter of about 5 to about 200  $\mu\text{m}$ . In one embodiment, the second particles 32 may have a substantially spherical particle shape. In another embodiment, the second particles 32 may comprise substantially non-spherical particles, including irregularly shaped particles, having rounded edges.

The metal coating layer 40 of a metal coating material 42 disposed on the outer surfaces 26 of the first metal particles 22 or the outer surfaces 36 of the second particles 32, or both, as described above, may be any suitable metal coating material 42 that is configured to provide a potential difference with the matrix 50 of first metal particles 22 as described herein. In one embodiment, the metal coating layer 40 includes a single metal layer. In this embodiment, the metal coating material 42 may include Al, Ni, Fe, Cu, In, Ga, Mn, Zn, Mg, Mo, Ca, Co, Ta, W, Si, or Re, or an alloy thereof, or any combination thereof. In other embodiments, the metal coating layer 40 may include a plurality of metal coating layers. In this embodiment, an inner layer is disposed on the metal coated powder particle (e.g. first metal particle 22, second particle 32 or both particles), and an outer layer is disposed over the inner layer. In one embodiment, the inner layer 46 may include Fe, Co, Cu, or Ni, or an alloy thereof, or a combination of any of the aforementioned inner layer materials, and the outer layer comprises Al, Zn, Mn, Mg, Mo, W, Cu, Fe, Si, Ca, Co, Ta, Re, or Ni, or an alloy thereof, or an oxide, nitride or carbide thereof, or a combination of any of the aforementioned outer layer materials. In another embodiment, the inner layer may include Al, Zn, Mn, Mg, Mo, W, Cu, Fe, Si, Ca, Co, Ta, Re, or Ni, or an alloy thereof, or an oxide, nitride or carbide thereof, or a combination of any of the aforementioned inner layer materials, and the outer layer may include Fe, Co, Cu, or Ni, or an alloy thereof, or a combination of any of the

forementioned outer layer materials. In one embodiment, where the first metal particles 22 include a magnesium-base alloy, the metal coating material includes Ni, Fe, Cu, or Co, or an alloy thereof, or any combination thereof. The metal coating layers 40 may have any suitable thickness, including a thickness of about 0.1 to about 10  $\mu\text{m}$ , and more particularly a thickness of about 1 to about 5  $\mu\text{m}$ . The difference in the oxidation potential between the first metal particles 22 and the metal coating layers 40 may be 10 any suitable oxidation potential difference, including a predetermined difference, and may be selected to provide a predetermined or selected dissolution or corrosion rate of the lightweight, high strength selectively degradable composite material 100. This may include the differences in the chemical compositions and oxidation potential difference may be 15 configured to provide a selectable and controllable dissolution rate, including a selectable transition from a very low dissolution rate to a very rapid dissolution rate, in response to a controlled change in a property or condition of the 20 wellbore proximate the powder compact material 110, including a property change in a wellbore fluid 6 that is in contact with the powder compact material 110, as described herein. In one embodiment, the first particle oxidation potential is about 0.7 volts or more, and the coating oxidation potential is about 0.5 volts or less. In other embodiments, a difference between the first particle oxidation potential and the coating oxidation potential is about 0.7 to about 2.7 volts.

The powder compact materials 110 disclosed herein may 30 be configured, including a difference between the first particle oxidation potential and the coating oxidation potential as described herein, to be selectively and controllably disposable, degradable, dissolvable, corrodible, or otherwise removable from a wellbore using a predetermined wellbore 35 fluid 6, including those described herein. These materials may, for example, be configured to be selectively dissolvable at a rate that ranges from about 0 to about 7000  $\text{mg/cm}^2/\text{hr}$  depending on the powder compact material 110 and wellbore fluid 6 selected. For example, the powder compact 40 material 100 may be selected to have a temperature dependent corrosion rate in a given wellbore fluid 6, such as a relatively low rate of corrosion in a 3% KCl solution at room temperature that ranges from about 0 to about 10  $\text{mg/cm}^2/\text{hr}$  as compared to relatively high rates of corrosion at 200° F. 45 in the same solution that range from about 1 to about 250  $\text{mg/cm}^2/\text{hr}$  depending on powder compact material 110 selected. An example of a changed condition comprising a change in chemical composition includes a change in a chloride ion concentration or pH value, or both, of the wellbore fluid 6. For example, various powder compact 50 materials 110 described herein may have corrosion rates in 15% HCl that range from about 4,500  $\text{mg/cm}^2/\text{hr}$  to about 7,500  $\text{mg/cm}^2/\text{hr}$ . Thus, selectable and controllable dissolvability in response to a changed condition in the wellbore, 55 namely the change in the wellbore fluid 6 chemical composition from KCl to HCl, may be achieved.

The lightweight, high strength, selectively degradable composite material 100 is a powder compact material 110 that may be formed into any article 200 by any suitable metalworking or forming method. Powder compact 100 may have any desired shape or size, including that of a cylindrical billet, bar, sheet or other form that may be machined, formed or otherwise used to form useful articles of manufacture, including various wellbore tools and components. Pressing 60 may be used to form a precursor powder compact 120 and sintering and pressing processes may be used to form powder compact 100 and deform the first metal powder

particles 22, second particles and coating layer 40, to provide the full density and desired macroscopic shape and size of powder compact 100 as well as its microstructure 50. The morphology (e.g. equiaxed or substantially elongated) of the deformed the first metal powder particles 22, second particles 32 and coating layer 40 results from sintering and deformation of these elements powder particles 12 as they are compacted and interdiffuse and deform to fill the inter-particle spaces. The sintering temperatures and pressures may be selected to ensure that the density of powder compact 110 achieves substantially full theoretical density.

In an exemplary embodiment, the microstructure 50 is formed at a sintering temperature ( $T_s$ ), where  $T_s$  is less than the melting temperature of the metal coating layer ( $T_c$ ) and the melting temperature of the first metal particle 22 ( $T_{p1}$ ) and second particle 32 ( $T_{p2}$ ). A solid-state metallurgical bond is formed in the solid state by solid-state interdiffusion between the metal coating layers 40 of adjacent metal coated particles, whether first metal particles 22, second particles, or both, that are compressed into touching contact during the compaction and sintering processes used to form powder compact 100, as described herein. As such, sintered metal coating layers 40 of network 56 include a solid-state bond layer that has a thickness defined by the extent of the interdiffusion of the coating materials 42 of the metal coating layers 40, which will in turn be defined by the nature of the coating layers 40, including whether they are single or multilayer coating layers, whether they have been selected to promote or limit such interdiffusion, and other factors, as described herein, as well as the sintering and compaction conditions, including the sintering time, temperature and pressure used to form powder compact 100.

As the network 56 of metal coating layers 40 is formed, including the metallurgical bond and bond layer, the chemical composition or phase distribution, or both, of metal coating layers 40 may change. Network 56 also has a melting temperature ( $T_m$ ). As used herein,  $T_m$  includes the lowest temperature at which incipient melting or liquation or other forms of partial melting will occur within network 56, regardless of whether the metal coating material 42 comprises a pure metal, an alloy with multiple phases each having different melting temperatures or a composite, including a composite comprising a plurality of layers of various coating materials having different melting temperatures, or a combination thereof, or otherwise. As the matrix 52 and dispersed particles 54 are formed in conjunction with network 56, diffusion of constituents of metallic coating layers 40 into the first metal particles 22 and/or second particles 32 is also possible, which may result in changes in the chemical composition or phase distribution, or both, of first metal particles 22 and/or second particles 32. As a result, matrix 52, network 56, dispersed particles 54 may have a melting temperature ( $T_{dp}$ ) that is different than  $T_p$ . As used herein,  $T_{dp}$  includes the lowest temperature at which incipient melting or liquation or other forms of partial melting will occur within matrix 52, regardless of whether metal first particle material that forms the matrix 52 comprises a pure metal, an alloy with multiple phases each having different melting temperatures or a composite, or otherwise. In one embodiment, powder compact 110 is formed at a sintering temperature ( $T_s$ ), where  $T_s$  is less than  $T_c$ ,  $T_p$ ,  $T_m$  and  $T_{dp}$ , and the sintering is performed entirely in the solid-state resulting in a solid-state bond layer. In another exemplary embodiment, powder compact material 110 is formed at a sintering temperature ( $T_s$ ), where  $T_s$  is greater than or equal to one or more of  $T_c$ ,  $T_p$ ,  $T_m$  or  $T_{dp}$  and the sintering includes limited or partial melting within

the powder compact material 110 as described herein, and further may include liquid-state or liquid-phase sintering resulting in a bond layer that is at least partially melted and resolidified. In this embodiment, the combination of a predetermined  $T_s$  and a predetermined sintering time ( $t_s$ ) will be selected to preserve the desired microstructure 50 as described herein. For example, localized liquation or melting may be permitted to occur, for example, within all or a portion of network 56 so long as the network, matrix 52 and dispersed particle 54 structure and morphology is preserved, such as by selecting first metal particles 22,  $T_s$  and  $t_s$  that do not provide for complete melting of the first metal particles 22. Similarly, localized liquation may be permitted to occur, for example, within all or a portion of matrix 52 so long as the microstructure 50 morphology is preserved, such as by selecting metal coating layers 40,  $T_s$  and  $t_s$  that do not provide for complete melting of the coating layer or layers 40. Melting of metal coating layers 40 may, for example, occur during sintering along the metal coating layer 40/first metal particle 22 interface, or along the interface between adjacent layers of multi-layer metal coating layers 40. It will be appreciated that combinations of  $T_s$  and  $t_s$  that exceed the predetermined values may result in other microstructures 50, such as an equilibrium melt/resolidification microstructure 50 if, for example, both the network 56 (i.e., combination of metal coating layers 40) and matrix 52 (i.e., the first metal particles 22) are melted, thereby allowing rapid interdiffusion of these materials.

The powder compact 110 is formed by a method that includes selecting the first metal particles 22 and the second particles 32. The method also includes coating at least one of the first metal particles 22 and the second particles 32 with a metal coating layer 40. The method also includes mixing the first metal particles 22 and the second particles 32 to form the powder mixture 10. Mixing may be performed to provide a homogeneous mixture 10 or a non-homogeneous or heterogeneous mixture as described herein. Mixing to provide a homogeneous powder mixture may be performed in any suitable mixing apparatus, including Attritor mixers, drum mixers, ball mills, blenders, including conical blenders, and the like, and by any suitable mixing method. In one embodiment, mixing was performed in an Attritor mixer having a central vertical shaft and one or more blending arms disposed thereon, such as a plurality of lateral extending axially and vertically spaced arms or a laterally and axially disposed helical arm. The Attritor mixer was water cooled and the mixing chamber purged with an inert gas during mixing. The powders are disposed therein together with a milling medium, such as ceramic or stainless steel beads having a diameter of about 6 to about 10 mm, while the shaft or mixing chamber is rotated for a predetermined mixing interval to mix or blend the powders and form the desired powder mixture 10. The mixing interval may be any suitable period, and in one embodiment may be about 10 to about 90 minutes, and more particularly about 30 to about 60 minutes. The method also includes forming the powder compact 110 with microstructure 50 from the powder mixture 10. The microstructure 50 formed of the network 56 of sintered metal coating layers 40, matrix 52 and dispersed particles 54 is formed by the compaction and sintering of the plurality of metal coating layers 40, first metal particles 22 and second particles 32, such as by CIP, HIP or dynamic forging. In one embodiment, the powder mixture may be compacted without sintering such that the microstructure comprises mechanical bonds between first metal particles 22, second particles 32 and metal coating layers 40 formed by deformation during compaction. The chemical composi-

tion of the network **56** may be different than that of metal coating material due to diffusion effects associated with the sintering. Powder metal compact **110** also includes matrix **52** that comprise first metal particles **22**. Network **56** and matrix **52** correspond to and are formed from the plurality of metal coating layers **40** and first metal particles **22**, respectively, as they are sintered together. The chemical composition of matrix **52** may also be different than that of first metal particles **22** due to diffusion effects associated with sintering. The method may also include forming an article **200** from the powder compact **110** by any suitable forming method as disclosed herein.

In one embodiment, the article **200** includes a selectively degradable article **210**. In another embodiment, the article **200** includes a selectively degradable downhole article **220**. In yet another embodiment, the selectively degradable downhole article **220** comprises a selectively degradable flow inhibition tool **230** or component **240**. In still further embodiments, the selectively degradable flow inhibition tool **230** or component **240** comprises a frac plug, bridge plug, wiper plug, shear out plug, debris barrier, atmospheric chamber disc, swabbing element protector, sealbore protector, screen protector, beaded screen protector, screen basepipe plug, drill in stim liner plug, inflow control device plug, flapper valve, gaslift valve, transmatic plug, float shoe, dart, diverter ball, shifting/setting ball, ball seat, plug seat, dart seat, sleeve, teleperf disk, direct connect disk, drill-in liner disk, fluid loss control flapper, shear pin, screw, bolt, or cement plug.

#### EXAMPLE

An example of the lightweight, high strength, selectively degradable composite material **100** and powder mixture **10** used to form it is described below and illustrated in FIGS. **5A-6**. A substantially homogeneous powder mixture **10** of a first powder **20** and second powder **30** was prepared by mixing in a ball mill for 60 min. The powder mixture **10** is shown in FIG. **5A**. The first metal particles **22** of first powder **20** comprise an Mg alloy having the nominal alloy composition, in weight percent of the alloy, 6 percent Zn, 1 percent Zr, and the balance Mg. The Mg alloy was prepared by gas atomization. The first metal particles **22** had an average particle diameter of 110  $\mu\text{m}$ . The first metal particles **22** had a uniform metal coating layer **40** that was 4  $\mu\text{m}$  thick. The second particles **32** comprise silicon carbide particles having an average particle diameter of 60  $\mu\text{m}$ . The powder mixture **10** comprised, in weight percent of the mixture, 39% of the first metal particles **22**, 60% of the second particles **32** and 1% of the metal coating layer **40**. The powder mixture **10** was compacted at 60 ksi and 450-500° C. by dynamic forging to substantially full theoretical density. The microstructure **50** is shown in the electron photomicrograph of FIG. **5B**. FIG. **5B** is a backscattered electron photomicrograph at 800x magnification showing the matrix **52** of first metal particles **22**, dispersed particles **54** of second particles **32** and the network **56** of metal coating layers **40**. The network **56** in this embodiment may be characterized as discontinuous, and more particularly as partially continuous. The powder compact material **110** of FIG. **5B** had the stress-strain characteristics in compression shown in the curve of FIG. **5C**.

In another embodiment, a different mixture of the particles described above having a reduced amount of first metal particles **22** and increased amount of second particles **32** was compacted under similar temperature and pressure conditions to form a powder compact **110** having the micro-

structure **50** shown in FIG. **6**. FIG. **6** is a secondary electron photomicrograph showing the matrix **52** of first metal particles **22**, dispersed particles **54** of second particles **32** and the network **56** of metal coating layers **40**. The network **56** of metal coating layers **40** may be characterized in this embodiment as locally continuous. FIG. **6** is an electron photomicrograph of the microstructure **50**. The microstructure **50** of the lightweight, high strength, selectively degradable composite material **100** has a UCS of about 97 ksi and is selectively degradable in a wellbore fluid **6** comprising a solution of 3% KCl in water at 98° C. at a rate of about 13.5 mg/cm<sup>2</sup>/hr, and in a different wellbore fluid **6** comprising a solution of 15% HCl in water at 98° C. at a rate of about 5000 mg/cm<sup>2</sup>/hr.

The terms “a” and “an” herein do not denote a limitation of quantity, but rather denote the presence of at least one of the referenced items. The modifier “about” used in connection with a quantity is inclusive of the stated value and has the meaning dictated by the context (e.g., includes the degree of error associated with measurement of the particular quantity). Furthermore, unless otherwise limited all ranges disclosed herein are inclusive and combinable (e.g., ranges of “up to about 25 weight percent (wt. %), more particularly about 5 wt. % to about 20 wt. % and even more particularly about 10 wt. % to about 15 wt. %” are inclusive of the endpoints and all intermediate values of the ranges, e.g., “about 5 wt. % to about 25 wt. %, about 5 wt. % to about 15 wt. %”, etc.). The use of “about” in conjunction with a listing of constituents of an alloy composition is applied to all of the listed constituents, and in conjunction with a range to both endpoints of the range. Finally, unless defined otherwise, technical and scientific terms used herein have the same meaning as is commonly understood by one of skill in the art to which this invention belongs. The suffix “(s)” as used herein is intended to include both the singular and the plural of the term that it modifies, thereby including one or more of that term (e.g., the metal(s) includes one or more metals). Reference throughout the specification to “one embodiment”, “another embodiment”, “an embodiment”, and so forth, means that a particular element (e.g., feature, structure, and/or characteristic) described in connection with the embodiment is included in at least one embodiment described herein, and may or may not be present in other embodiments.

It is to be understood that the use of “comprising” in conjunction with the alloy compositions described herein specifically discloses and includes the embodiments wherein the alloy compositions “consist essentially of” the named components (i.e., contain the named components and no other components that significantly adversely affect the basic and novel features disclosed), and embodiments wherein the alloy compositions “consist of” the named components (i.e., contain only the named components except for contaminants which are naturally and inevitably present in each of the named components).

While one or more embodiments have been shown and described, modifications and substitutions may be made thereto without departing from the spirit and scope of the invention. Accordingly, it is to be understood that the present invention has been described by way of illustrations and not limitation.

The invention claimed is:

1. A lightweight, selectively degradable composite material comprising
  - a compacted powder mixture of
  - a first powder, the first powder comprising first metal particles comprising Mg, Al, Mn, or Zn, or an alloy of

## 17

any of the above, or a combination of any of the above, having a first metal particle oxidation potential, the first particles having an average size of about 75 to about 150 microns, and a second powder, the second powder comprising low-density ceramic, glass, cermet, intermetallic, metal, polymer, or inorganic compound second particles, the first metal particles comprising a metal coating layer of a coating material disposed on an outer surface having a coating oxidation potential that is different than the first metal particle oxidation potential, the first metal particles comprising about 10 to about 50 percent, and the second particles comprising about 50 to about 90 percent, by weight of the composite material, the compacted powder mixture having a microstructure comprising:

a matrix comprising the first metal particles; the second particles dispersed within the matrix; and a network comprising interconnected adjoining metal coating layers and having a length of about 2 to about 10 times the diameters of the first metal particles, the lightweight, selectively degradable composite material having a density of about  $3.5 \text{ g/cm}^3$  or less.

2. The composite material of claim 1, wherein both of the first metal particles and the second particles have the metal coating layer disposed on the outer surfaces.

3. The composite material of claim 1, wherein the second particles comprise pure Ti or a Ti alloy.

4. The composite material of claim 1, wherein the lightweight, selectively degradable composite material has a density of about 1.5 to about  $3.5 \text{ g/cm}^3$ .

5. The composite material of claim 1, wherein the first metal particle oxidation potential is about 0.7 volts or more, and the coating oxidation potential is about 0.5 volts or less.

6. The composite material of claim 1, wherein a difference between the first metal particle oxidation potential and the coating oxidation potential is about 0.7 to about 2.7 volts.

7. The composite material of claim 1, wherein the composite material has an ultimate compressive strength of at least 80 ksi.

8. The composite material of claim 1, wherein the composite material has an ultimate compressive strength of at least 100 ksi.

9. The composite material of claim 1, wherein the first metal particles comprise a magnesium-base alloy.

10. The composite material of claim 9, wherein the magnesium-base alloy comprises an Mg—Si, Mg—Al, Mg—Zn, Mg—Mn, Mg—Al—Zn, Mg—Al—Mn, Mg—Zn—Zr, or Mg—X alloy, where X comprises a rare earth element, or an alloy thereof, or any other combination of the aforementioned.

11. The composite material of claim 10, wherein the coating material comprises Ni, Fe, Cu, or Co, or an alloy thereof, or any combination thereof.

12. The composite material of claim 1, wherein the second particles have a density of about 0.1 to about  $4.0 \text{ g/cm}^3$ .

13. The composite material of claim 1, wherein the second particles comprise hollow metal particles.

14. The composite material of claim 1, wherein the second particles have an average particle size of about 10 to about 200  $\mu\text{m}$ .

15. The composite material of claim 1, wherein the ceramic, glass, polymer, or inorganic compound second particles are porous.

## 18

16. The composite material of claim 1, wherein the ceramic particles comprise metal carbide, nitride, or oxide particles, or a combination thereof.

17. The composite material of claim 1, wherein the second particles comprise uncoated silicon carbide particles.

18. The composite material of claim 17, wherein the silicon carbide particles have an average diameter of about 5 to about 200  $\mu\text{m}$ .

19. The composite material of claim 1, wherein the coating material comprises Al, Ni, Fe, Cu, In, Ga, Mn, Zn, Mg, Mo, Ca, Co, Ta, W, Si, or Re, or an alloy thereof, or any combination thereof.

20. The composite material of claim 1, wherein the coating layer has a thickness of about 0.1 to about 10  $\mu\text{m}$ .

21. The composite material of claim 1, wherein the coating layer has a thickness of about 1 to about 5  $\mu\text{m}$ .

22. The composite material of claim 1, wherein the metal coating layer is disposed only on the first metal particles.

23. The composite material of claim 1, wherein the first metal particles comprise about 15 to about 50 percent by weight of the composite material, the second particles comprise about 50 to about 85 percent by weight of the composite material, and the coating layers comprise about 0.5 to about 5 percent by weight of the composite material.

24. The composite material of claim 1, wherein the metal coating layer comprises a plurality of metal coating layers.

25. The composite material of claim 24, wherein an inner layer is disposed on the second particles, and an outer layer is disposed over the inner layer, and wherein the inner layer comprises Fe, Co, Cu, or Ni, or an alloy thereof, or a combination of any of the aforementioned inner layer materials, and the outer layer comprises Al, Zn, Mn, Mg, Mo, W, Cu, Fe, Si, Ca, Co, Ta, Re, or Ni, or an alloy thereof, or an oxide, nitride or carbide thereof, or a combination of any of the aforementioned outer layer materials.

26. The composite material of claim 24, wherein an inner layer is disposed on the at least one of the first metal particles and the second particles, and an outer layer is disposed over the inner layer, and wherein the inner layer comprises Al, Zn, Mn, Mg, Mo, W, Cu, Fe, Si, Ca, Co, Ta, Re, or Ni, or an alloy thereof, or an oxide, nitride or carbide thereof, or a combination of any of the aforementioned inner layer materials, and the outer layer comprises Fe, Co, Cu, or Ni, or an alloy thereof, or a combination of any of the aforementioned outer layer materials.

27. The composite material of claim 1, wherein the second particles comprise substantially spherical particles.

28. The composite material of claim 1, wherein the second particles comprise substantially non-spherical particles having rounded edges.

29. The composite material of claim 1, wherein the second powder comprises low-density polymer second particles.

30. The composite material of claim 1, wherein the network is locally continuous and extends only to metal coating layers of immediately adjacent first metal particles or to a cluster of 10 or less immediately adjacent first metal particles.

31. A lightweight, selectively degradable composite material comprising  
a compacted powder mixture of  
a first powder, the first powder comprising first metal particles comprising Mg, Al, Mn, or Zn, or an alloy of any of the above, or a combination of any of the above, having a first metal particle oxidation potential, and

**19**

a second powder, the second powder comprising hollow or porous low-density ceramic, cermet, intermetallic, metal, polymer, or inorganic compound second particles,

the second particles having an average particle size of about 10 to about 200  $\mu\text{m}$  and comprising a metal coating layer of a coating material disposed on an outer surface having a coating oxidation potential that is different than the first metal particle oxidation potential,

the first metal particles comprising about 10 to about 50 percent, and the second particles comprising about 50 to about 90 percent, by weight of the composite material,

the compacted powder mixture having a microstructure comprising:

a matrix comprising the first metal particles; the second particles dispersed within the matrix; and a network comprising interconnected adjoining metal coating layers and having a length of about 2 to about 10 times the diameters of the second metal particles, the lightweight, selectively degradable composite material having a density of about  $3.5 \text{ g/cm}^3$  or less, and wherein the coating layer is disposed only on the second particles.

**32.** A selectively degradable article, comprising:  
a lightweight, selectively degradable composite material, the composite material comprising a compacted powder mixture of  
a first powder, the first powder comprising first metal particles comprising Mg, Al, Mn, or Zn, or an alloy of any of the above, or a combination of any of the above, having a first metal particle oxidation potential, and  
a second powder, the second powder comprising low-density ceramic, glass, cermet, intermetallic, metal, polymer, or inorganic compound second particles,

**20**

the first metal particles comprising a metal coating layer of a coating material disposed on an outer surface having a coating oxidation potential that is different than the first metal particle oxidation potential, the first metal particles comprising about 10 to about 50 percent, and the second particles comprising about 50 to about 90 percent, by weight of the composite material,

the compacted powder mixture having a microstructure comprising:

a matrix comprising the first metal particles; the second particles dispersed within the matrix; and a network comprising interconnected adjoining metal coating layers and having a length of about 2 to about 10 particle diameters of the first metal particles, the lightweight, selectively degradable composite material having a density of about  $3.5 \text{ g/cm}^3$  or less.

**33.** The article of claim **32**, wherein the composite material comprises a selectively degradable downhole article.

**34.** The article of claim **33**, wherein the selectively degradable downhole article comprises a selectively degradable flow inhibition tool or component.

**35.** The article of claim **34**, wherein the selectively degradable flow inhibition tool or component is selected from the group consisting of a frac plug, bridge plug, wiper plug, shear out plug, debris barrier, atmospheric chamber disc, swabbing element protector, sealbore protector, screen protector, beaded screen protector, screen basepipe plug, drill in stim liner plug, inflow control device plug, flapper valve, gaslift valve, transmatic plugs, float shoe, dart, diverter ball, shifting/setting ball, ball seat, plug seat, dart seat, sleeve, teleperf disk, direct connect disk, drill-in liner disk, fluid loss control flapper, shear pin, screw, bolt, and cement plug.

**36.** A method of at least partially inhibiting flow in a wellbore using the article of claim **34**.

\* \* \* \* \*